# EUROPEAN PATENT SPECIFICATION

(11) **EP 1 605 080 B1**
(45) Date of publication and mention of the grant of the patent: **02.04.2008**
(21) Application number: 05102899.1
(22) Date of filing: 13.04.2005
(51) Int. Cl.: D02G 3/40, D02G 3/44, D01F 8/14

(54) **Woven papermaking fabric**
Papiermaschinengewebe
Tissu pour machine à papier

(30) Priority: 21.05.2004 US 850684; 12.11.2004 US 986167
(43) Date of publication of application: 14.12.2005
(73) Proprietor: Voith Patent GmbH, 89522 Heidenheim (DE)
(72) Inventor: Payne, Dwight, 31522, St. Simons Island (US); Ross, Gilbert, 31503, Waycross (US); Zhang, Heping, 29483, Summerville (US); Morton, Antony, LS298QU, Ilkley (GB); Craig, Valentine, 29485, Summerville (US)

(56) References cited:
- EP-A- 0 361 758
- EP-A- 0 676 297
- EP-A- 1 188 852
- EP-A- 1 316 634
- DE-A1- 4 404 507
- GB-A- 2 221 477
- US-A- 4 126 499
- US-A- 4 467 839
- US-A- 4 876 774
- US-A- 5 294 482
- US-A- 5 534 335
- US-A- 5 615 713
- US-A- 6 117 548

## Description

### FIELD OF INVENTION

The present invention relates to yarns made of polymeric material for use in industrial fabrics.

### DESCRIPTION OF PRIOR ART

Industrial fabrics, especially papermaking fabrics, are typically but not exclusively made of a woven structure using polymer yarns in the weft and warp direction. To improve the smoothness and the printability of a paper sheet produced on a papermaking fabric it is desirable to increase the smoothness and the contact area of the paper contacting surface of the papermaking fabric. Especially for high speed applications it is further desirable to increase the smoothness of the wear side of the papermaking fabric in order to improve the aerodynamic performance of the fabric.

The smoothness of the paper contacting surface can be improved by increasing the yarn density resulting in increased manufacturing costs and reduced permeability of the fabric.

Further the smoothness can be improved by using profiled monofilament yarns having flat surface. When using the flat shaped yarns, e.g. as warp yarns in float weave designs, the flat warp yarns provide greater surface contact area. It has been found that for many application the gain in contact area by using such flat yarns is not sufficient. Especially for graphic and fine paper grades it would be desirable to bring the weft yarns as well as the warp yarns into the paper contacting surface of the papermaking fabric to increase the contact area and the smoothness of the fabric to a sufficient level.

### SUMMARY OF THE INVENTION

It is the object of the present invention to provide a papermaking fabric with which it is possible to overcome the disadvantages described above.

According to the invention there is provided a woven papermaking fabric including at least in part yarns made from a polymeric material, wherein the industrial fabric has been subjected to a heat set temperature during production, wherein the polymeric material includes a first phase and a second phase, and wherein the melting temperature of the second phase is equal or less than the heat set temperature and wherein the melting temperature of the first phase is higher than the heat set temperature.

Therefore, at least some weft and/or warp yarns of the papermaking fabric are made of polymeric material having two phases.

The papermaking fabric, preferably is a forming or a dryer fabric.

The idea of the invention is to provide a papermaking fabric with yarns having the ability for controllable deformation when subjected to mechanical tension and thermal heat, as is the case during heat set treatment for industrial fabrics. The yarn used for the fabric according to the invention is therefore made from a polymeric material including two different phases which have two different melting points wherein the melting temperature of the second phase is equal or less than the maximum heat set temperature and wherein the melting temperature of the first phase is higher than the maximum heat set temperature.

The second phase takes over the part that the yarn softens during heat set treatment and the first phase take over the part that the yarn does not melt. Therefore by combining a first and second polymeric phase according to the invention a yarn is provided which softens during the heat set treatment and becomes very deformable without melting.

If the yarns including polymeric material with two phases are e.g. weft yarns of the fabric and if the warp yarns of the fabric are made from standard yarn material, during heat set treatment the harder warp yarns can compress the softer and deformable weft yarns resulting in a crimp interchange between the warps and the wefts leading to a reduction of the warp knuckles giving a fabric with enhanced surface smoothness.

Typical maximum heat set temperatures are in the range of 90°C to 260°C.

Further the papermaking fabric will be operated on a papermaking machine at a maximum operation temperature. Therefore according to a preferred embodiment of the invention the melting temperature of the second phase is higher than the maximum operating temperature.

According to a preferred embodiment of the invention the polymeric material is a polymer blend wherein the first phase includes a first polymer component and wherein the second phase includes a second polymer component and wherein the first and the second polymer component are at least substantially immiscible. By blending immiscible polymer compounds most of the properties, e.g. the melting temperature of each polymer compound, will be maintained substantially.

It is further possible that the first and the second phase are of the same material and differ in their state of aggregation.

Depending on the application the maximum operation temperature for the papermaking fabric is less than 90°C or less 120°C. For papermaking fabrics maximum heat set temperatures are in the ranges as follows: Forming fabrics: 170°C to 190°C, typically 180°C to 185°C Press fabrics: 160°C to 185°C, typically 160°C to 165°C Dryer fabrics: 180°C to 220°C, typically 190°C Therefore the melting temperature of the second phase / second polymer component is in the range of 120°C to 220°C, preferably in the range of 160°C to 220°C.

### By way of example:

A fabric will be subjected to a heat set treatment with a maximum temperature of 190°C and will be operated at a maximum operation temperature of 120°C. Therefore the melting temperature of the second phase of a yarn according to the invention must be lower than 190°C and higher than 120°C. The melting temperature of the first phase of this yam is more than 190°C.

According to a further preferred embodiment of the invention the melting temperature of the second phase / second polymer component is at least 30°C lower than the melting temperature of the first phase / first polymer component.

According to a further preferred embodiment of the invention the melting temperature of the second phase / second polymer component is at least 80°C lower than the melting temperature of the first phase / first polymer component.

According to another preferred embodiment of the invention the melting temperature of the second phase / second polymer component is typically between 100°C and 110°C lower than the melting temperature of the first phase / first polymer component.

Further the first component includes any of the following either alone or blended: homopolymers and copolymers of the polyesters, homopolymers and-copolymers of polyamides, PPS.

Most preferably the first component includes PET.

In addition the second component includes any of the following either alone or blended: polyolefins, polyamides, fluoropolymers.

Most preferably the second component includes Polyolefins.

It has been found by the applicant that yarns for use in a papermaking fabric according to the invention showing the best deformability at the heat set temperature for which they are designed is a blend including between 51% and 99% by weight, preferably between 60% and 95% by weight, of the first component and between 49% and 1% by weight, preferably between 5% and 40% by weight, of the second component.

To allow the polymer blend to be processed it may be necessary to incorporate at least one suitable compatibilizer. Without a suitable compatibilizer e.g. mechanical properties, e.g. toughness of the yarn produced can be reduced. Further for immiscible polymer blends the so called "die swell" during extrusion can increase which effects the controllability of the extruded yarn diameter. Therefore according to a further preferred embodiment the polymer blend includes at least one suitable compatibilizer.

It has been found by the applicant the best results in regard to processability can be achieved if the at least one compatibilizer is included in an amount of 0,01% to 10% by weight, preferably in an amount of 0,1 to 5% by weight.

There are different types of compatibilizer suitable for the polymer blend according to the invention. According to a preferred embodiment of the invention at least one compatibilizer is a physical compatibilizer. A physical compatibilizer is based on the principle that components of the compatibilizer are miscible which each component / phase of the blend. Thus the compatibilizer is acting as a polymeric surfactant.

According to a further preferred embodiment of the invention the physical compatibilizer is any of the following: Ethylene Methyl Acrylate Copolymer (EMA), Ethylene Butyl Acrylate Copolymer (EBA). By way of example the blend includes the polymer components PE and PET and the compatibilizer EMA. In this case the ethylene component of the compatibilizer is miscible with PE and the methacrylate component of the compatibilizer is miscible with PET.

A suitable compatibilizer also can be a reactive compatibilizer. This method of compatibilization relies e.g. on the chemical reaction between the functional group that is grafted onto the PE and the end groups of the PET. This results in the in-situ formation of a PET/PE copolymer which then acts as a physical compatibilizer for the blend.

The suitable reactive compatibilizer can be any of the following: Ethylene -g- Maleic Anhydride Copolymers, Ethylene - g- Glycidal Methacrylate.

Further the polymer blend can include at least one suitable stabilizer. A stabilizer for example is added to design yarns with the ability to withstand severe conditions as high temperature and / or high humidity. According to one preferred embodiment of the present invention the at least one stabilizer is a hydrolysis stabilizer. Hydrolysis stabilizers are added to the blend to generate yarns for the use under high humidity conditions.

The hydrolysis stabilizer can be a carbodiimide compound either monomeric, polymeric or a combination.

According to a further preferred embodiment of the invention the at least one stabilizer can be an anti-oxidation stabilizer. Anti-oxidation stabilizers are added to the blend to generate yarns for the use under high temperature conditions.

It has been found by the applicant that the best results in retaining the properties of the blend can be achieved if the at least one stabilizer is included in an amount of 0,1% to 10% by weight, preferably in an amount of 0,5 to 5% by weight.

Further the two phase polymeric yarn for use in the fabric according to the invention preferably is a monofilament yarn but also can be a multifilament yarn.

The papermaking fabric can comprise two phase yarns with a diameter in the range of 0,20mm to 2,0mm, preferable in the range of 0,4mm to 1,0mm. These diameters are suitable for most of the different types of papermakers fabrics.

According to a further embodiment of the invention the shape of the yarn is round or profiled e.g. with chamfered edges.

It has been found by the applicant that an industrial fabric not forming part of the invention comprising a set of weft yarns and a set of warp yarns, where in the warp yarns and the weft yarns are interwoven to form a specific weave design, and wherein tension has been applied to said weft yarns or said warp yarns during a heat set treatment, has improved surface smoothness and wear resistance if at least one of said yarns of said fabric not have been tensioned during heat set treatment has an enhanced crimp level of at least 0,5% compared to the corresponding yarn of a reference fabric, wherein said reference fabric has the same weave design as said fabric, wherein all weft and warp yarns of said reference fabric have the same diameter as said weft and warp yarns of said fabric, wherein said reference fabric has been manufactured under the same conditions as said fabric, and wherein said corresponding not tensioned yarn of said reference fabric is made from PET based polymeric material.

By providing a fabric comprising yarns which haven 't been tensioned during heat set treatment and which have after heat set treatment an enhanced crimp level of at least 0,5% compared to yarns made from PET having the same position in a reference fabric as said yarns in said fabric, wherein said reference fabric being identical in all features and in manufacturing as said fabric according to the invention except that said similar / corresponding yarns are made from PET, said non tensioned yarns and said tensioned yarns of said fabric lie more together in one common plane of said fabric compared to the yarns in the reference fabric. This leads to a fabric according to the invention having enhanced smoothness, less tendency of wire marking and improved wear resistance.

The crimp level is calculated with the following formula: $( length along the crimped line of the yarn - length along the straight line of the yarn ) / length along the straight line of the yarn * 100 = crimp level in %$

By way of example for a given yam the length along the crimped line of the yarn is 12 cm and the length along the straight line is 10 cm the crimp level is (12cm-10cm)/10cm *100 = 20%.

Preferably, at least some of said yarns not being tensioned during heat set treatment have the enhanced crimp level compared to said corresponding yarns in said reference fabric.

Most preferably all of said yarns no tension has been applied to during heat set treatment have the enhanced crimp level.

Preferably said non tensioned yarns are weft yarns.

It has been found by the applicant that the enhanced level of crimp is at least 1,0%, preferably at least 1,5%, most preferably in the range of 1,5% to 2,5%. It has been found that with increasing crimp level the smoothness of the fabric increases. Further it has been found that an optimum in smoothness is achieved if the crimp level of said non tensioned yarns during heat set treatment is in the range of 1,5% and 2,5%.

Typical heat set conditions are:
- tension selected from the range of 1kN/m to 6kN/m,
- temperature with a maximum temperature selected from the range of 90°C to 260°C.

Further it has been found by the applicant that the paper contacting surface has an enhanced smoothness over the paper contacting surfaces of prior art papermaking fabrics leading to less sheet marking if the ratio of crimp level of the warp yarns to the crimp level of the weft yarns is as low as possible.

The above described behaviour will be explained by way of example as follows: During heat set treatment tension and temperature is applied to the warp yarns. At least some of the weft yarns are made from a material which softens at the maximum heat set temperature and therefore is very deformable at the maximum heat set temperature. Further the warp yarns are made from a material which softens less than the weft yarns at the maximum heat set temperature. The fact that the weft yarns are made from the material which softens more during heat set treatment than the warp yarns allows the harder warp yarns to compress the softer weft yarns reducing the warp knuckles leading to a smoother fabric.

Based on the discussion from below it is therefore desirable if the ratio of the crimp level of at least one warp yarn to the crimp level of at least one weft yarn is less than 3,5, preferably less than 3,0, most preferably less than 2.

In the case of a dryer fabric the dryer fabric has an air permeabitlity in the range from 50 to 200cfm, preferably in the range from 75 to 150cfm.

According to a preferred embodiment in regard to a specific weave design the industrial fabric the set of wet yarns comprises first and second weft yarns, wherein said first weft yarns are disposed over said second weft yarns and wherein said warp yarns weave over two consecutive first weft yarns before weaving under one second weft yarn. It has been found by the applicant that a weave design according to this embodiment has improved surface smoothness.

According to a embodiment of the above mentioned weave design said first weft yarns are in offset position relative to said second weft yarns.

According to another embodiment of said weave design it is foreseen that adjacent warp yarns weave in offset position relative to each other over said two consecutive first weft yarns, wherein the offset position of said adjacent warp yarns preferably is at least one first weft yarn.

Preferably the weave design comprise per weave repeat four warp yarns and four first and four second weft yarns.

The following examples are intended to illustrate the invention, not to limit it.

**Table 1:**

| Composition | Reference | Sample1 | Sample 2 | Sample 3 | Sample 4 |
|---|---|---|---|---|---|
| | | | | | |
| Component 1 | 100% PET | 98% PET | 95% PET | 91 % PET | 87,3% PET |
| | | | | | |
| Component 2 | --- | 2% PE | 5% PE | 5% PE | 5% PE |
| | | | | | |
| Additive 1 | --- | --- | --- | 1% Anti-Oxidant | 0,5% Anti-Oxidant |
| | | | | | |
| Additive 2 | --- | --- | --- | 3% Compatibilizer | 3% Compatibilizer |
| | | | | | |
| Additive 3 | --- | --- | --- | --- | 1,2% Hydrolysis stabilizer |
| | | | | | |
| Melting temp. phase 1 [°C] | 253 | 253 | 253 | 253 | 253 |
| | | | | | |
| Melting temp. phase 2 [°C] | --- | 120 | 120 | 120 | 120 |
| | | | | | |
| Tenacity [gpd] | 2,9 | 3,1 | 2,9 | 2,8 | 3,1 |
| | | | | | |
| Elongation at break [%] | 45 | 47 | 46 | 54 | 45 |
| | | | | | |
| Young's Modulus [gpd] | 72 | 71 | 70 | 63 | 60 |
| | | | | | |
| Shrinkage [%] | 15 | 15,8 | 17 | 12 | 11 |
| | | | | | |
| Strength retained [%] after hydrolysis at 140°C, 24hours | 69 | 63 | 38 | 30 | 85 |
| | | | | | |
| Strength retained [%] after dry heat at 204°C, 24hours | 46 | 44 | 51 | 54 | 80 |

All the different components are added in % age by weight.

Table 1 is showing a comparison between a standard PET monofilament yam (Reference) and monofilament yarns according to the invention (Sample 1 to Sample 4) having the same yarn diameter (0,7mm) as the reference yarn.

As can be seen in table 1 the yarns of samples 1 to 4 have two melting temperatures. A melting temperature of the first phase which is at 253°C and a melting temperature of 120°C of the second phase. Therefore the yam according to the invention has a melting temperature (120°C) which is in the temperature range of typical heat set treatments (90°C to 220°C) and a melting temperature which is higher than the heat set temperature.

Sample 1 to 4 are made from a polymer blend including the polymer components PET and PE, wherein the first phase is formed by the PET polymer component and the second phase is formed by the PE polymer component. PET and PE are immiscible polymers and therefore generate a blend with two phases.

As can be seen especially sample 1,2 and 4 have approximately the same mechanical properties as the reference sample. Sample 1 has the same degradation resistance as the reference sample.

To improve the processability samples 3 and 4 include 3% of a compatibilizer.

To improve the resistance to dry heat treatment sample 3 further includes 1% of an anti -oxidation stabilizer. As can be seen the strength retained after dry heat treatment is increased to 54%.

To improve hydrolysis resistance sample 4 further includes a hydrolysis stabilizer in an amount of 1,2%. As can be seen from table 1 sample 4 has the best dry heat and wet heat resistance behaviour.

The invention shall be further illustrated with the following figures, wherein
- Figure 1: shows a comparison between the paper contacting surface of a dryer fabric made from standard yarn material and a dryer fabric made from yam material according to the invention,
- Figure 2: shows the difference in contact area between the dryer fabric according to the invention and a standard dryer fabric,
- Figure 3: shows the difference in crimp level between the dryer fabric according to the invention and a standard dryer fabric,
- Figure 4: shows a preferred weave design in warp yarn direction of a fabric for use with the yarns according to the invention.

Figure 1 shows a photograph of the paper contacting surface of a dryer fabric 1 made from standard yarn material and a photograph of the paper contacting surface of a dryer fabric 10 made from yam material according to the invention.

It has to be noted that both fabrics 1, 10 have the same weave design and that the weft and the warp yarns of both fabrics have the same diameter. Further both fabrics are manufactured identically at least in terms of the heat set treatment which had been performed applying a tension in the range of 1,5kN/m to 5kN/m to the warp yarns with a temperature in the range of 170°C to 220°C.

Figure 1 a shows the paper contacting surface 2 of the fabric 1 having warp 3 and weft 4 yarns made from 100% PET.

Figure 1 b shows the paper contacting surface 11 of the fabric 10 having warp yarns 12 made from 100% PET and having weft yarns 13 made from a PET-PE polymer blend according to the invention.

As can be seen in Figure 1 a the weft yarns 4 of the fabric 1 substantially extend in a straight line having a low crimp level. Measurement have shown a crimp level in the 4% range. In contrast thereto the warp yarns 3 have a high crimp level which is approximately 19%. Therefore the paper contacting surface of the dryer fabric 1 only has a contact area of 22% (grey coloured) as shown in Figure 2 a. further the crimp level ratio of warp yam to weft yarn is 4,75.

As can be seen in Figure 1 b the weft yarns 13 of the fabric 10 extend in a crimped line having a high crimp level compared with the crimp level of the weft yarns 4 according to Figure 1 a. Measurement have shown a crimp level of the wefts 13 is in the 5,5% range. Further the warp yarns 12 have a lower crimp level than the warp yarns 3 of the dryer fabric 1. The crimp level of the warps 12 is approximately 10%. Therefore the paper contacting surface of the dryer fabric 10 has an enhanced contact area 14 of 30% (grey coloured) as shown in Figure 2 b compared to the contact area 5 of the dryer fabric 1 which is 22% (grey coloured) as shown in Figure 2 a. According to the invention the crimp level ratio of warp yam to weft yam is 1,8.

Figure 3 shows the difference in crimp level between a weft yam 13 of the dryer fabric 10 according to the invention and a weft yarn 4 of the standard dryer fabric 1.

A weft yarn of a fabric according to the invention can have a crimp level in the range of 5,0% to 7,0%, typically in the range of 5,5% to 6,5%, depending on the specific weave design, the yarn diameter and the heat set conditions.

The weft yarns 13 of the fabric 10 has a crimp level of 6,0%.

A weft yarn of a fabric known in the art can have a crimp level in the range of 3,5% to 5,5%, typically in the range of 4,0% to 5,0%, depending on the specific weave design, the yarn diameter and the heat set conditions.

The weft yarns 4 of the fabric 1 has a crimp level of 4,0%.

For the same weave design and the same manufacturing conditions the weft yarns of a fabric according to the invention has an enhanced crimp level of at least 0,5%, preferably at least 1,0%, most preferably at least 1,5% and prefered in the range of 1,5% to 2,5%.

In the concrete embodiment of Figure 1 the difference in crimp level between fabric 10 and 1 is 2%.

Figure 4 shows the weave design of fabrics 1 and 10 in warp yarn direction. For the further discussion the weave design will be discussed by reference numbers of fabric 10.

Fabric 10 comprises first weft yarns 13a, 13b, 13c, 13d and second weft yarns 13e, 13f, 13g and 13h. The first weft yarns 13a, 13b, 13c, 13d are disposed over said second weft yarns 13e, 13f, 13g and 13h. Further first weft yarns 13a, 13b, 13c, 13d are in offset position relative to second weft yarns 13e, 13f, 13g and 13h.

As can be seen warp yarns 12A, 12B, 12C and 12D weave over two consecutive first weft yarns before weaving under one second weft yarn.

By way of example warp yarn 12B (dashed line) weaves over consecutive first weft yams 13a and 13b before weaving under second weft yam 13h.

In addition adjacent warp yarns weave in offset position relative to each other over said two consecutive first weft yarns, wherein the offset position is defined by one first weft yam.

By way of example warp yam 12B weaves over first weft yarns 13a and 13b, wherein adjacent warp yarn 12C (dash dotted line) weaves over first weft yarns 13b and 13c. Therefore the offset between warp yarn 12B and Warp yam 12C is defined by one first weft yarn.

As can be seen the weave repeat comprises four warp yarns 12A to 12D and four first weft yarns 13a, 13b, 13c, 13d and four second weft yarns 13e, 13f, 13g 13h.

## Claims

1. Woven papermaking fabric (10) including yarns (12, 13), wherein the fabric (10) has been subjected to heat set treatment during manufacture,
**characterized in**
**that** the fabric (10) includes at least in part yarns (13) made from a polymeric material, said polymeric material includes a first phase having a melting temperature and a second phase having a melting temperature, the melting temperature of the second phase is equal or less the maximum heat set temperature and that the melting temperature of the first phase is higher than the maximum heat set temperature.

2. Woven papermaking fabric according to claim 1,
**characterized in**
**that** the maximum heat set temperature is selected from the range of 90°C and 260°C.

3. Woven papermaking fabric according to claim 1 or 2,
**characterized in**
**that** the woven papermaking fabric (10) will be operated at a maximum operation temperature, wherein the melting temperature of the second phase is higher than the maximum operation temperature.

4. Woven papermaking fabric according to one of the preceding claims,
**characterized in**
**that** second phase is an amorphous phase and that the melting temperature of the amorphous second phase is a softening temperature.

5. Woven papermaking fabric according to one of the preceding claims,
**characterized in**
**that** the polymeric material is a polymer blend wherein the first phase includes a first polymer component and wherein the second phase includes a second polymer component and wherein the first and the second polymer component are substantially immiscible.

6. Woven papermaking fabric according to one of the preceding claims,
**characterized in**
**that** the melting temperature of the second phase / second polymer component is in the range of 120°C to 220°C, preferably in the range of 160°C to 220°C.

7. Woven papermaking fabric according to one of the preceding claims ,
**characterized in**
**that** the melting temperature of the second phase / second polymer component is at least 30°C lower than the melting temperature of the first phase / first polymer component.

8. Woven papermaking fabric according to claim 7 ,
**characterized in**
**that** the melting temperature of the second phase / second polymer component is at least 80°C lower than the melting temperature of the first phase / first polymer component.

9. Woven papermaking fabric according to claim 7 or 8,
**characterized in**
**that** the melting temperature of the second phase / second polymer component is typically between 100°C and 110°C lower than the melting temperature of the first phase / first polymer component.

10. Woven papermaking fabric according to one of the preceding claims,
**characterized in**
**that** the first component includes any of the following either alone or blended: homepolymers and copolymers of the polyesters, homepolymers and copolymers of polyamides, PPS.

11. Woven papermaking fabric according to claim 10,
**characterized in**
**that** the first component includes PET.

12. Woven papermaking fabric according to one of the preceding claims,
**characterized in**
**that** the second component includes any of the following either alone or blended: polyolefins, polyamides, fluoropolymers.

13. Woven papermaking fabric according to one of the preceding claims,
**characterized in**
**that** the blend includes between 51% and 99% by weight, preferably between 60% and 95% by weight, of the first component and between 49% and 1% by weight, preferably between 5% and 40% by weight, of the second component.

14. Woven papermaking fabric according to one of the preceding claims,
**characterized in**
**that** the polymer blend comprises at least one suitable compatibilizer.

15. Woven papermaking fabric according to claim 14,
**characterized in**
**that** the at least one compatibilizer is included in an amount of 0,01% to 10% by weight, preferably in an amount of 0,1 to 5% by weight.

16. Woven papermaking fabric according to one of the preceding claims,
**characterized in**
**that** the at least one compatibilizer is a physical compatibilizer.

17. Woven papermaking fabric according to claim 16,
**characterized in**
**that** the physical compatibilizer is any of the following: Ethylene Methyl Acrylate Copolymer (EMA), Ethylene Butyl Acrylate Copolymer.

18. Woven papermaking fabric according to one of the preceding claims,
**characterized in**
**that** the at least one compatibilizer is a reactive compatibilizer.

19. Woven papermaking fabric according to claim 18,
**characterized in**
**that** the reactive compatibilizer is any of the following: Ethylene -g- Maleic Anhydride Copolymers, Ethylene - g- Glycidal Methacrylate.

20. Woven papermaking fabric according to one of the preceding claims,
**characterized in**
**that** the polymer blend comprises at least one suitable stabilizer.

21. Woven papermaking fabric according to claim 20,
**characterized in**
**that** the at least one stabilizer is included in an amount of 0,1 % to 10% by weight, preferably in an amount of 0,5 to 5% by weight.

22. Woven papermaking fabric according to claim 20 or 21,
**characterized in**
**that** the at least one stabilizer is a hydrolysis stabilizer.

23. Woven papermaking fabric according claim 22,
**characterized in**
**that** the hydrolysis stabilizer is a carbodiimide compound.

24. Woven papermaking fabric according to claim 20 or 21,
**characterized in**
**that** the at least one stabilizer is an anti-oxidation stabilizer.

25. Woven papermaking fabric according to one of the preceding claims,
**characterized in**
**that** the yarn (13) is a monofilament yarn.

26. Woven papermaking fabric according to one of the preceding claims,
**characterized in**
**that** the yam is a multifilament yarn.

27. Woven papermaking fabric according to one of the preceding claims,
**characterized in**
**that** the yarn (13) has a diameter in the range of 0,20mm to 2,0mm, preferable in the range of 0,4mm to 1,0mm.

28. Woven papermaking fabric according to one of the preceding claims,
**characterized in**
**that** the shape of the yarn (13) is round or profiled e.g. with chamfered edges.

29. Woven papermaking fabric according to one of the claims 1 to 28,
**characterized in**
**that** the dryer fabric has an air permeability in the range from 50 to 200cfm, preferably in the range from 75 to 150cfm.

30. Woven papermaking fabric according to one of the claims 1 to 29,
**characterized in**
**that** said set of wet yarns comprises first and second weft yarns, said first weft yarns being disposed over said second weft yarns and wherein said warp yarns weave over two consecutive fist weft yarns before weaving under one second weft yarn.

31. Woven papermaking fabric according to claim 30,
**characterized in**
**that** said first weft yarns are in offset position relative to said second weft yarns.

32. Woven papermaking fabric according to claim 30 or 31,
**characterized in**
**that** adjacent warp yarns weave in offset position relative to each other over said two consecutive first weft yarns.

33. Woven papermaking fabric according to claim 32,
**characterized in**
**that** said offset position of said adjacent warp yarns is at least one first weft yarn.

34. Woven papermaking fabric according to one of the claims 30 to 33,
**characterized in**
**that** the weave repeat comprises four warp yarns and four first and four second weft yarns.

35. Woven papermaking fabric according to one of the claims 30 to 34,
**characterized in**
**that** the weft yarns have the enhanced level of crimp.

## Patentansprüche

1. Papiermaschinengewebe (10) mit Garnen (12, 13), wobei das Gewebe (10) während der Herstellung einer Thermofixierbehandlung unterzogen wurde,
**dadurch gekennzeichnet,**
**dass** das Gewebe (10) wenigstens zum Teil Garne (13) beinhaltet, die aus einem Polymermaterial hergestellt sind, das Polymermaterial eine erste Phase mit einer Schmelztemperatur und eine zweite Phase mit einer Schmelztemperatur beinhaltet, die Schmelztemperatur der zweiten Phase gleich oder niedriger ist als die maximale Thermofixiertemperatur und dass die Schmelztemperatur der ersten Phase höher ist als die maximale Thermofixiertemperatur.

2. Papiermaschinengewebe nach Anspruch 1,
**dadurch gekennzeichnet,**
**dass** die maximale Thermofixiertemperatur im Bereich von 90°C bis 260°C gewählt wird.

3. Papiermaschinengewebe nach Anspruch 1 oder Anspruch 2,
**dadurch gekennzeichnet,**
**dass** das Papiermaschinengewebe (10) mit einer maximalen Betriebstemperatur betrieben werden wird, wobei die Schmelztemperatur der zweiten Phase höher ist als die maximale Betriebstemperatur.

4. Papiermaschinengewebe nach einem der vorhergehenden Ansprüche,
**dadurch gekennzeichnet,**
**dass** die zweite Phase eine amorphe Phase ist und dass die Schmelztemperatur der amorphen zweiten Phase eine Erweichungstemperatur ist.

5. Papiermaschinengewebe nach einem der vorhergehenden Ansprüche
**dadurch gekennzeichnet,**
**dass** das Polymermaterial ein Polymerblend ist, wobei die erste Phase eine erste Polymerkomponente beinhaltet und die zweite Phase eine zweite Polymerkomponente beinhaltet und wobei die erste Polymerkomponente und die zweite Polymerkomponente im Wesentlichen unmischbar sind.

6. Papiermaschinengewebe nach einem der vorhergehenden Ansprüche,
**dadurch gekennzeichnet,**
**dass** die Schmelztemperatur der zweiten Phase / zweiten Polymerkomponente im Bereich von 120°C bis 220°C, vorzugsweise im Bereich von 160°C bis 220°C, liegt.

7. Papiermaschinengewebe nach einem der vorhergehenden Ansprüche,
**dadurch gekennzeichnet,**
**dass** die Schmelztemperatur der zweiten Phase / zweiten Polymerkomponente mindestens 30°C niedriger ist als die Schmelztemperatur der ersten Phase / ersten Polymerkomponente.

8. Papiermaschinengewebe nach Anspruch 7,
**dadurch gekennzeichnet,**
**dass** die Schmelztemperatur der zweiten Phase / zweiten Polymerkomponente mindestens 80°C niedriger ist als die Schmelztemperatur der ersten Phase / ersten Polymerkomponente.

9. Papiermaschinengewebe nach Anspruch 7 oder Anspruch 8,
**dadurch gekennzeichnet,**
**dass** die Schmelztemperatur der zweiten Phase / zweiten Polymerkomponente typischerweise 100°C bis 110°C niedriger ist als die Schmelztemperatur der ersten Phase / ersten Polymerkomponente.

10. Papiermaschinengewebe nach einem der vorhergehenden Ansprüche,
**dadurch gekennzeichnet,**
**dass** die erste Komponente Folgendes entweder allein oder als Gemisch beinhaltet: Homopolymere und Copolymere der Polyester, Homopolymere und Copolymere von Polyamiden, PPS.

11. Papiermaschinengewebe nach Anspruch 10,
**dadurch gekennzeichnet,**
**dass** die erste Komponente PET beinhaltet.

12. Papiermaschinengewebe nach einem der vorhergehenden Ansprüche,
**dadurch gekennzeichnet,**
**dass** die zweite Komponente Folgendes entweder allein oder als Gemisch beinhaltet: Polyolefine, Polyamide, Fluorpolymere.

13. Papiermaschinengewebe nach einem der vorhergehenden Ansprüche,
**dadurch gekennzeichnet,**
**dass** das Blend 51 Gew.-% bis 99 Gew.-%, vorzugsweise 60 Gew.-% bis 95 Gew.-%, der ersten Komponente und 49 Gew.-% bis 1 Gew.-%, vorzugsweise 5 Gew.-% bis 40 Gew.-%, der zweiten Komponente beinhaltet.

14. Papiermaschinengewebe nach einem der vorhergehenden Ansprüche,
**dadurch gekennzeichnet,**
**dass** das Polymerblend wenigstens einen geeigneten Verträglichkeitsvermittler beinhaltet.

15. Papiermaschinengewebe nach Anspruch 14,
**dadurch gekennzeichnet,**
**dass** der wenigstens eine Verträglichkeitsvermittler in einer Menge von 0,01 bis 10 Gew.-%, vorzugsweise in einer Menge von 0,1 bis 5 Gew.-%, enthalten ist.

16. Papiermaschinengewebe nach einem der vorhergehenden Ansprüche,
**dadurch gekennzeichnet,**
**dass** der wenigstens eine Verträglichkeitsvermittler ein physikalischer Verträglichkeitsvermittler ist.

17. Papiermaschinengewebe nach Anspruch 16,
**dadurch gekennzeichnet,**
**dass** der physikalische Verträglichkeitsvermittler einer der folgenden Stoffe ist: Ethylen-Methylacrylat-Copolymer (EMA), Ethylen-Butylacrylat-Copolymer.

18. Papiermaschinengewebe nach einem der vorhergehenden Ansprüche,
**dadurch gekennzeichnet,**
**dass** der wenigstens eine Verträglichkeitsvermittler ein reaktiver Verträglichkeitsvermittler ist.

19. Papiermaschinengewebe nach Anspruch 18,
**dadurch gekennzeichnet,**
**dass** der reaktive Verträglichkeitsvermittler einer der folgenden Stoffe ist: Ethylen-g-Maleinsäureanhydrid-Copolymere, Ethylen-g-Glycidylmethacrylat.

20. Papiermaschinengewebe nach einem der vorhergehenden Ansprüche,
**dadurch gekennzeichnet,**
**dass** das Polymerblend wenigstens einen geeigneten Stabilisator beinhaltet.

21. Papiermaschinengewebe nach Anspruch 20,
**dadurch gekennzeichnet,**
**dass** der wenigstens eine Stabilisator in einer Menge von 0,1 bis 10 Gew.-%, vorzugsweise in einer Menge von 0,5 bis 5 Gew.-%, enthalten ist.

22. Papiermaschinengewebe nach Anspruch 20 oder Anspruch 21,
**dadurch gekennzeichnet,**
**dass** der wenigstens eine Stabilisator ein Hydrolysestabilisator ist.

23. Papiermaschinengewebe nach Anspruch 22,
**dadurch gekennzeichnet,**
**dass** der Hydrolysestabilisator eine Carbodiimid-Verbindung ist.

24. Papiermaschinengewebe nach Anspruch 20 oder Anspruch 21,
**dadurch gekennzeichnet,**
**dass** der wenigstens eine Stabilisator ein Antioxidationsstabilisator ist.

25. Papiermaschinengewebe nach einem der vorhergehenden Ansprüche,
**dadurch gekennzeichnet,**
**dass** das Garn (13) ein Monofilgarn ist.

26. Papiermaschinengewebe nach einem der vorhergehenden Ansprüche,
**dadurch gekennzeichnet,**
**dass** das Garn ein Multifilgarn ist.

27. Papiermaschinengewebe nach einem der vorhergehenden Ansprüche,
**dadurch gekennzeichnet,**
**dass** das Garn (13) einen Durchmesser im Bereich von 0,20 mm bis 2,0 mm, vorzugsweise im Bereich von 0,4 mm bis 1,0 mm, aufweist.

28. Papiermaschinengewebe nach einem der vorhergehenden Ansprüche,
**dadurch gekennzeichnet,**
**dass** das Garn (13) eine runde Form oder eine profilierte Form, z. B. mit abgeschrägten Kanten, aufweist.

29. Papiermaschinengewebe nach einem der Ansprüche 1 bis 28,
**dadurch gekennzeichnet,**
**dass** das Trockensieb eine Luftdurchlässigkeit im Bereich von 50 bis 220 cfm, vorzugsweise im Bereich von 75 bis 150 cfm, aufweist.

30. Papiermaschinengewebe nach einem der Ansprüche 1 bis 29,
**dadurch gekennzeichnet,**
**dass** der Satz von Schussfäden erste und zweite Schussfäden aufweist, wobei die ersten Schussfäden über den zweiten Schussfäden angeordnet sind und wobei die Kettfäden zuerst über zwei aufeinander folgenden ersten Schussfäden verlaufen und dann unter einem zweiten Schussfäden verlaufen.

31. Papiermaschinengewebe nach Anspruch 30,
**dadurch gekennzeichnet,**
**dass** die ersten Schussfäden in Bezug auf die zweiten Schussfäden jeweils versetzt angeordnet sind.

32. Papiermaschinengewebe nach Anspruch 30 oder Anspruch 31,
**dadurch gekennzeichnet,**
**dass** benachbarte Kettfäden versetzt zueinander über die jeweils zwei aufeinander folgenden ersten Schussfäden verlaufen.

33. Papiermaschinengewebe nach Anspruch 32,
**dadurch gekennzeichnet,**
**dass** die benachbarten Kettfäden zueinander um jeweils wenigstens einen ersten Schussfaden versetzt sind.

34. Papiermaschinengewebe nach einem der Ansprüche 30 bis 33,
**dadurch gekennzeichnet,**
**dass** der Bindungsrapport vier Kettfäden und vier erste und vier zweite Schussfäden umfasst.

35. Papiermaschinengewebe nach einem der Ansprüche 30 bis 34,
**dadurch gekennzeichnet,**
**dass** die Schussfäden den erhöhten Kräuselungsgrad aufweisen.

## Revendications

1. Tissu tissé pour machine à papier (10) comprenant des fils (12, 13), dans lequel le tissu (10) a été soumis à un traitement de thermofixage pendant la fabrication, **caractérisé en ce que** le tissu (10) comprend au moins en partie des fils (13) fabriqués à partir d'un matériau polymère, ledit matériau polymère comprenant une première phase avec une température de fusion et une seconde phase avec une température de fusion, la température de fusion de la seconde phase étant égale ou inférieure à la température de thermofixage maximale et la température de fusion de la première phase étant supérieure à la température de thermofixage maximale.

2. Tissu tissé pour machine à papier selon la revendication 1, **caractérisé en ce que** la température de thermofixage maximale est choisie dans la plage de 90 °C à 260 °C.

3. Tissu tissé pour machine à papier selon la revendication 1 ou la revendication 2, **caractérisé en ce que** le tissu tissé pour machine à papier (10) sera utilisé à une température de fonctionnement maximale, dans lequel la température de fusion de la seconde phase est supérieure à la température de fonctionnement maximale.

4. Tissu tissé pour machine à papier selon l'une quelconque des revendications précédentes, **caractérisé en ce que** la seconde phase est une phase amorphe et **en ce que** la température de fusion de la seconde phase amorphe est une température de ramollissement.

5. Tissu tissé pour machine à papier selon l'une quelconque des revendications précédentes, **caractérisé en ce que** le matériau polymère est un mélange polymère dans lequel la première phase comprend un premier composant polymère et dans lequel la seconde phase comprend un second composant polymère et dans lequel le premier et le second composant polymère sont essentiellement non miscibles.

6. Tissu tissé pour machine à papier selon l'une quelconque des revendications précédentes, **caractérisé en ce que** la température de fusion de la seconde phase / second composant polymère se situe dans la plage de 120 °C à 220 °C, de préférence dans la plage de 160 °C à 220 °C.

7. Tissu tissé pour machine à papier selon l'une quelconque des revendications précédentes, **caractérisé en ce que** la température de fusion de la seconde phase / second composant polymère est d'au moins 30 °C inférieure à la température de fusion de la première phase / premier composant polymère.

8. Tissu tissé pour machine à papier selon la revendication 7, **caractérisé en ce que** la température de fusion de la seconde phase / second composant polymère est d'au moins 80 °C inférieure à la température de fusion de la première phase / premier composant polymère.

9. Tissu tissé pour machine à papier selon la revendication 7 ou la revendication 8, **caractérisé en ce que** la température de fusion de la seconde phase / second composant polymère est de 100 °C à 110 °C inférieure à la température de fusion de la première phase / premier composant polymère.

10. Tissu tissé pour machine à papier selon l'une quelconque des revendications précédentes, **caractérisé en ce que** le premier composant comprend l'un quelconque des éléments suivants seul ou mélangé : homopolymères et copolymères de polyesters, homopolymères et copolymères de polyamides, PPS.

11. Tissu tissé pour machine à papier selon la revendication 10, **caractérisé en ce que** le premier composant comprend du PET.

12. Tissu tissé pour machine à papier selon l'une quelconque des revendications précédentes, **caractérisé en ce que** le second composant comprend l'un quelconque des éléments suivants seul ou mélangé : polyoléfines, polyamides, fluoropolymères.

13. Tissu tissé pour machine à papier selon l'une quelconque des revendications précédentes, **caractérisé en ce que** le mélange comprend entre 51 % et 99 % en poids, de préférence entre 60 % et 95 % en poids, du premier composant et entre 49 % et 1 % en poids, de préférence entre 5 % et 40 % en poids, du second composant.

14. Tissu tissé pour machine à papier selon l'une quelconque des revendications précédentes, **caractérisé en ce que** le mélange polymère comprend au moins un agent de compatibilité approprié.

15. Tissu tissé pour machine à papier selon la revendication 14, **caractérisé en ce qu'**au moins un agent de compatibilité est compris en une quantité de 0,01 % à 10 % en poids, de préférence en une quantité de 0,1 à 5 % en poids.

16. Tissu tissé pour machine à papier selon l'une quelconque des revendications précédentes, **caractérisé en ce qu'**au moins un agent de compatibilité est un agent de compatibilité physique.

17. Tissu tissé pour machine à papier selon la revendication 16, **caractérisé en ce que** l'agent de compatibilité physique est l'un des suivants : copolymère d'acrylate d'éthylène-méthyle (EMA), copolymère d'acrylate d'éthylène-butyle.

18. Tissu tissé pour machine à papier selon l'une quelconque des revendications précédentes, **caractérisé en ce qu'**au moins un agent de compatibilité est un agent de compatibilité réactif.

19. Tissu tissé pour machine à papier selon la revendication 18, **caractérisé en ce que** l'agent de compatibilité réactif est l'un des suivants : copolymères d'éthylène-g-anhydride maléique, éthylène-g-méthacrylate de glycidal.

20. Tissu tissé pour machine à papier selon l'une quelconque des revendications précédentes, **caractérisé en ce que** le mélange polymère comprend au moins un stabilisant approprié.

21. Tissu tissé pour machine à papier selon la revendication 20, **caractérisé en ce qu'**au moins un stabilisant est compris en une quantité de 0,1 % à 10 % en poids, de préférence en une quantité de 0,5 à 5 % en poids.

22. Tissu tissé pour machine à papier selon la revendication 20 ou la revendication 21, **caractérisé en ce qu'**au moins un stabilisant est un stabilisant d'hydrolyse.

23. Tissu tissé pour machine à papier selon la revendication 22, **caractérisé en ce que** le stabilisant d'hydrolyse est un composé à base de carbodiimide.

24. Tissu tissé pour machine à papier selon la revendication 20 ou la revendication 21, **caractérisé en ce qu'**au moins un stabilisant est un stabilisant anti-oxydation.

25. Tissu tissé pour machine à papier selon l'une quelconque des revendications précédentes, **caractérisé en ce que** le fil (13) est un fil monofilament.

26. Tissu tissé pour machine à papier selon l'une quelconque des revendications précédentes, **caractérisé en ce que** le fil (13) est un fil multifilament.

27. Tissu tissé pour machine à papier selon l'une quelconque des revendications précédentes, **caractérisé en ce que** le fil (13) a un diamètre dans la plage de 0,20 mm à 2,0 mm, de préférence dans la plage de 0,4 mm à 1,0 mm.

28. Tissu tissé pour machine à papier selon l'une quelconque des revendications précédentes, **caractérisé en ce que** la forme du fil (13) est ronde ou profilée, par ex., avec des bords chanfreinés.

29. Tissu tissé pour machine à papier selon l'une quelconque des revendications 1 à 28, **caractérisé en ce que** le tissu sécheur possède une perméabilité à l'air dans la plage de 50 à 200 pi³/min, de préférence dans la plage de 75 à 150 pi³/min.

30. Tissu tissé pour machine à papier selon l'une quelconque des revendications 1 à 29, **caractérisé en ce que** ledit ensemble de fils de trame comprend des premiers et des seconds fils de trame, lesdits premiers fils de trame étant disposés par-dessus lesdits seconds fils de trame et dans lequel desdits fils de chaîne sont tissés par-dessus deux premiers fils de trame consécutifs avant d'être tissés sous un second fil de trame.

31. Tissu tissé pour machine à papier selon la revendication 30, **caractérisé en ce que** lesdits premiers fils de trame sont dans une position décalée par rapport auxdits seconds fils de trame.

32. Tissu tissé pour machine à papier selon la revendication 30 ou la revendication 31, **caractérisé en ce que** les fils de chaîne adjacents sont tissés dans une position décalée les uns par rapport aux autres par-dessus lesdits deux premiers fils de trame consécutifs.

33. Tissu tissé pour machine à papier selon la revendication 32, **caractérisé en ce que** ladite position décalée desdits fils de chaîne adjacents est au moins un premier fil de trame.

34. Tissu tissé pour machine à papier selon l'une quelconque des revendications 30 à 33, **caractérisé en ce que** la répétition du tissage comprend quatre fils de chaîne et quatre premiers et quatre seconds fils de trame.

35. Tissu tissé pour machine à papier selon l'une quelconque des revendications 30 à 34, **caractérisé en ce que** les fils de trame possèdent un niveau accru de frisure.
